# EUROPEAN PATENT SPECIFICATION

(11) **EP 3 240 916 B1**
(45) Date of publication and mention of the grant of the patent: **18.09.2019**
(21) Application number: 15822955.9
(22) Date of filing: 28.12.2015
(51) Int. Cl.: C22C 1/05, C22C 19/05, C22C 29/06, C22C 29/02, C22C 29/08, B22F 3/15

(54) **LIGHT WEIGHT CEMENTED CARBIDE FOR FLOW EROSION COMPONENTS**
LEICHTES HARTMETALL FÜR FLUIDEROSIONSFESTE KOMPONENTEN
CARBURES CÉMENTÉS LÉGERS POUR COMPOSANTS SOUMIS À L'ÉROSION PAR FLUIDES

(30) Priority: 30.12.2014 US 201462098229 P
(43) Date of publication of application: 08.11.2017
(73) Proprietor: Hyperion Materials & Technologies (Sweden) AB, 126 80 Stockholm (SE)
(72) Inventor: DORVLO, Selassie, Olton Solihull B92 8RF (GB); KEOWN, Eugene, Bourton on Dunsmore CV23 9 RA (GB); SMITH, Jane, Coventry West Midlands CV6 IEL (GB); NORDENSTRÖM, Henrik, 136 66 Vendelsö (SE); MECH, Milena, Royal Leamington Spa CV32 4TR (GB); CARPENTER, Michael, Nuneaton Warwickshire CV10 0PF (GB)
(74) Representative: Neilson, Martin Mark
(86) International application number: PCT/EP2015/081284
(87) International publication number: WO 2016/107843

(56) References cited:
- EP-A1- 1 019 557
- EP-A1- 2 439 294
- EP-A1- 2 439 300
- EP-A2- 1 939 314
- WO-A1-01/14608
- GB-A- 1 350 634

## Description

### TECHNICAL FIELD/INDUSTRIAL APPLICABILITY

The present disclosure relates to cemented carbides for flow components, and more particularly to a flow control apparatus, fluid handling components and sealing rings with improved service life.

### BACKGROUND

Seal rings are the key critical component in mechanical shaft seals for pumps. Cemented carbides show a good mechanical performance in this kind of application. However, energy consumption and corrosion resistance is an issue in pumps. If the weight of the cemented carbide seal ring can be reduced, so will the energy consumption. A reduction in weight will also reduce the cost of the seal rings and in turn the cost of the pump.

One of the most important properties for seal rings is corrosion resistance. During operation of the pump, the seal surface will be exposed to the pumping media which can often be corrosive. Corrosion during life of a seal ring will lead to the binder being dissolved. This will lead to the increased wear of the seal ring. When this happens there will be a significant increase in the amount fluid leaking from the pump. There is need for a corrosion resistant cheaper tungsten carbide seal ring.

Similarly, cemented carbide flow components, the primary function of which is to control the pressure and flow of well products used in, for example, the oil and gas industry where components are subjected to high pressures of multi-media fluid where there is a corrosive environment.

Light-weight cemented carbide for improved service life of can punches is disclosed in EP2439294B1, assigned to the assignee of the present disclosure. The cemented carbide has a hard phase comprising WC and a binder phase, wherein the cemented carbide composition comprises, in wt-%, from 50 to less than 70 WC, from 15 to 30 TiC, and from 12 to 20 Co+Ni.

### SUMMARY

It is an aspect of the present disclosure to provide a cemented carbide for fluid handling components and seal rings having improved corrosion resistance.

In one aspect, the present disclosure relates to a cemented carbide for fluid handling components and seal rings comprising in wt %; 15 to 30 TiC; 5 to 20 Ni; 0.5 to 2.5 Cr₃C₂; 0.7 to 1.6 Mo and the remainder WC.

In an embodiment, the cemented carbide composition as defined hereinabove or hereinafter comprises from 20 to 23wt % TiC.

In an embodiment, the cemented carbide composition as defined hereinabove or hereinafter comprises from 0.8 to 1.5 wt % Cr₃C₂, such as about 0.95 to about 1.3 wt % Cr₃C₂.

In an embodiment, the cemented carbide composition as defined hereinabove or hereinafter comprises from 9.5 to 14.5 wt% Ni, such as about 10 to about 14 wt% Ni.

In an embodiment, the cemented carbide composition as defined hereinabove or hereinafter has an average WC grain size of from 0.9 µm to 1.3 µm, such as of about 1.05 µm to about 1.15 µm measured by FSSS. The foregoing summary, as well as the following detailed description of the embodiments, will be better understood when read in conjunction with the appended drawings. It should be understood that the embodiments depicted are not limited to the precise arrangements and instrumentalities shown.

### BRIEF DESCRIPTION OF THE DRAWINGS

Fig. 1 is an optical microscopy image of an illustrative example of a cemented carbide not forming part of the present invention.
Fig. 2 is a scanning electron microscope (SEM) image of the illustrative example of Fig. 1.
Fig. 3 is an SEM image of another illustrative example of a cemented carbide not forming part of the present invention of Fig. 1.
Fig. 4 is an SEM image of a comparative example not forming part of the present invention.
Fig. 5 is an SEM image of an embodiment of a cemented carbide according to a further illustrative example not forming part of the present invention.
Fig. 6 is an SEM image of an embodiment of a cemented carbide for a seal ring according to an aspect of the present invention.
Fig. 7 is an SEM image of another embodiment of a cemented carbide for a seal ring according to an aspect of the present invention.
Fig. 8 is an SEM image of another embodiment of a cemented carbide for a seal ring according to an aspect of the present invention.

### DETAILED DESCRIPTION

As used herein, the term "about" means plus or minus 10% of the numerical value of the number with which it is being used. Therefore, about 50% means in the range of 45%-55%.

As will be described fully herein, embodiments of the present disclosure relate to cemented carbides for flow components (herein, the term "component" means parts or pieces), particularly for seal rings and for choke trim components used in the oil and gas industry, where the components are subjected to high pressures of multi-media fluid and where there is a corrosive environment, particularly for choke valve components whose 10 primary function of which is to control the pressure and flow of well products, such as pumps. Under severe conditions of multi flow media; these components may suffer from extreme mass loss by exposure to solid particle erosion, acidic corrosion erosion-corrosion synergy and cavitation mechanisms even when fitted with cemented carbide trims. The components will also suffer due to galvanic corrosion due to a electropotential difference between the binder and the housing for the flow control part.

The light weight cemented material can also be used in, for example, seal rings, to reduce the weight of the seal ring. In order to improve the corrosion resistance the light weight cemented carbide of the present disclosure can have a Ni-Cr-Mo binder.

An illustrative example of a light weight cemented carbide for use in flow components not forming part of the present invention, such as seal rings, has a composition in wt % of about 15 to about 30 TiC, about 12 to about 20 Co + Ni, about 0.5 to about 2.5 Cr; and about 0.1 to about 0.3 Mo and the balance WC. The WC may have an average sintered grain size of about 0.5µm. The sintered structure is also shown in Figs. 1 and 2.

Seal rings are the key critical component in mechanical shaft seals for pumps. Cemented carbide show a good mechanical performance in this kind of application. The cemented carbide seal rings of the present disclosure have a reduced weight and therefore allow for less energy consumption. Furthermore, the cemented carbide seal rings have improved application relevant properties, such as improved corrosion resistance.

Referring to Fig. 1 (not forming part of the present invention), the cemented Carbide for a flow component, LW, as defined hereinabove or hereinafter and used, for example, in a flow control apparatus, has the following composition ranges in weight %: about 7 to about 9 wt% Co, about 5 to about 7 wt% Ni, about 19 to about 24 wt% TiC, about 1.5 to about 2.5 wt% Cr₃C₂, about 0.1 to about 0.3 wt % Mo and the balance WC.

The hardness of the cemented carbide component as defined hereinabove or hereinafter may be of from about 1350 to about 1500 HV30 (IS03878), the toughness (Klc) being about 8.5 to about 9.5 MPa ●√m by indentation technique according to Klc (SEVNB) >8.5 MPa ●√m and the transverse rupture strength (TRS) according to IS03327 type C>1700 N/mm².

The WC in the cemented carbide may have an average sintered grain size of about 0.8 µm and the (Ti,W)C (titanium tungsten carbide in the cemented carbide may have an average sintered grain size of about 1.5 µm according to IS04499-2-2010.

The carbon content within the sintered cemented carbide as defined hereinabove or hereinafter should be kept within a narrow range in order to retain a high resistance to corrosion and wear, as well as have a high toughness. The carbon level of the sintered structure is held in the lower portion of the range between free carbon in the microstructure (top limit) and eta-phase initiation (bottom limit).

Magnetic saturation measurements for the magnetic binder phase of the sintered cemented carbide is expressed in terms of µT m³ kg-1 and relate to the nature of the combined multi element binder. For the sintered material according to the disclosure, this should lie between 80 % and 90% of the 2-phase field of the binder. No eta-phase or graphite is permitted in the sintered structure. The sintered structure is shown in Fig. 1.

The re-passivity of the embodiment, depicted as LW is improved due to the significant addition of TiWC hard phase added to the composition. Corrosion resistance was determined using the ASTM G61. ASTM G61 covers a procedure for conducting potentiodynamic polarization measurements. See Table 1 below showing the results of ASTM G61 comparing an embodiment with a comparative example.

**Table 1: ASTM G61 Evaluated parameters from polarization curves**

| Product | Eb 10 µm/cm² | Eb 100 µm/cm² | Ereprass 10 µm/cm² |
|---|---|---|---|
| Comparative Example | 24 | 46 | -333 |
| LW | 118 | 156 | -76 |

"Eb" is the breakdown potential, at which localised corrosion occurs and is evaluated at two different criteria. The lower criterion of 10µA/cm² may be considered to give an indication of the ease of initiation of corrosion. The difference between this and the higher criterion of 100 µA/cm² provides an indication of the propagation process.

"Erepass" is the potential required to repassivate the specimen.

Conventional powder metallurgical methods such as milling, drying, pressing, shaping, sintering and sinter hipping, which are used for manufacture of conventional cemented carbides are used to manufacture the embodiments of the present disclosure.

### EXAMPLES

It should be appreciated that the following examples are illustrative, non-limiting example. The compositions and results of the embodiments are shown in Tables 2 and 3 below.

In the examples below the powders were sourced from the following suppliers: (W,Ti)C from Zhuzhou or HC Starck, Co from Umicore or Freeport, Ni from Inco, Mo from HC Starck and Cr₃C₂ from Zhuzhou or HC Starck

### Illustrative example 1 - not encompassed by the present invention ('LW flow control' - reference A)

Cemented carbide grades with the composition in wt-% 21 TiC; 8.3 Co; 5.7; Ni; 0.2 Mo and 2 Cr₃C₂ with the balance of WC was produced using WC and (Ti,W)C powder with an average FSSS particle size (d₅₀) of 0.8 µm and about 3 µm, respectively. The cemented carbide samples were prepared from powders forming the hard constituents and powders forming the binder. The powders were wet milled together with lubricant and anti -flocculating agent until a homogeneous mixture was obtained and granulated by drying. The dried powder was pressed on the Tox press to bodies and 'green machined' before sintering. Sintering was performed at 1360 -1410°C for about 1 hour in vacuum, followed by applying a high pressure, 50 bar Argon, at sintering temperature for about 30 minutes to obtain a dense structure before cooling.

The sintered cemented carbide structure comprises of some hexagonal WC with an average grain size of 0.8 µm together with (Ti,W)C grains with an average grain size of 1.5 µm as measured using the linear intercept method.

The material has a hardness of about 1350 to about 1500 HV30 depending on the selected composition and sinter temperature.

As shown in Fig. 3, the illustrative example of the cemented carbide disclosure, LW shows improved wear resistance to scratch testing in comparison to a comparative example of a fine grained oil and gas grade with 10.5wt% binder (Fig. 4) with similar or hardness values. Testing was carried out using a diamond Stylus with a 20 µm radius tip at 200 mN.

Wear resistance damage from scratching is considerably improved for the example of the disclosure, LW, as shown by reduced 'grey' amorphous damage in Fig. 3 as compared to the comparative example in Fig. 4. Further, corrosion resistance for the example of the disclosure, LW, in seawater is improved and with better repassivity (See Table 1).

The hardness of the cemented carbide component may be about 1350 to about 1500 HV30 (IS03878), the toughness (Klc) being about 8.7 MPa ●√m using Palmqvist toughness technique according to ISO28079 or Klc (LW15, SEVNB) > 8.5 MPa ●√m and the transverse rupture strength (TRS) according to IS03327 type C>1700 N/mm².

### Illustrative example 2 - not encompassed by the present invention ('LW seal ring' - reference B)

A cemented carbide grades with the compositions in wt-% of about 63.2 WC; about 20.8 TiC; about 2 Cr₃C₂; about 8.2 Co; about 5.6 Ni and about 0.2 Mo was produced using WC powder with an average FSSS particle grain size (d₅₀) of 4-8 µm, respectively. The sintered structure is shown in Figs. 5.

The cemented carbide samples were prepared from powders forming the hard constituents and powders forming the binder. The powders were wet milled together with lubricant and anti -flocculating agent until a homogeneous mixture was obtained and granulated by drying. The dried powder was pressed on the Tox press to bodies and 'green machined' before sintering. Sintering is performed at 1360 -1410°C for about 1 hour in vacuum, followed by applying a high pressure, 50 bar Argon, at sintering temperature for about 30 minutes to obtain a dense structure before cooling.

An embodiment of the light weight cemented carbide for seal rings according to the present disclosure, (LW + CR), has a composition of about 15 to about 30 wt% TiC, about 5 to about 20 wt% Ni, about 0.5 to about 2.5 wt% Cr, and about 0.7 to about 1.6 wt% Mo and the balance WC.

### Example 3 according to an aspect of the present invention ('LW + CR seal ring' - reference C)

A cemented carbide grades with the compositions in wt-% of about 66.04 WC; about 21.95 TiC; about 0.95 Cr₃C₂; about 0.95 Mo; about 10.11 Ni using WC and (Ti,W)C powder with an average FSSS particle size (d₅₀) of greater than about 1 µm, for example 1.1 and 1.15 µm, respectively. It should be appreciated that a particle size of up to about 8 µm can be used.

The sintered structure is shown in Fig. 6.

The cemented carbide samples were prepared from powders forming the hard constituants and powders forming the binder. The powders were wet milled together with lubricant and anti-flocculating agent until a homogeneous mixture was obtained and granulated by drying. The dried powder was pressed on the Tox press to bodies and 'green machined' before sintering. Sintering is performed at 1360 -1410°C for about 1 hour in vacuum, followed by applying a high pressure, 50 bar Argon, at sintering temperature for about 30 minutes to obtain a dense structure before cooling.

The hardness of the cemented carbide component may be about 1550 HV30 (IS03878), the toughness (Klc) being about 8.5 MPa ●√m using Palmqvist toughness technique according to ISO28079 and a density of about 10.2 g/cm³.

### Example 4 according to an aspect of the present invention ('LW + CR seal ring' - reference D)

A cemented carbide grades with the compositions in wt-% of about 62.79 WC; about 20.86 TiC; about 1.29 Cr₃C₂; about 1.29 Mo; about 13.78 Ni WC and (Ti,W)C powder with an average FSSS particle size (d₅₀) of greater than about 1 µm, for example 1.1 and 1.15 µm, respectively. It should be appreciated that a particle size of up to about 8 µm can be used.

The cemented carbide samples were prepared from powders forming the hard constituents and powders forming the binder. The powders were wet milled together with lubricant and anti-flocculating agent until a homogeneous mixture was obtained and granulated by drying. The dried powder was pressed on the Tox press to bodies and 'green machined' before sintering. Sintering is performed at 1360 -1410°C for about 1 hour in vacuum, followed by applying a high pressure, 50 bar Argon, at sintering temperature for about 30 minutes to obtain a dense structure before cooling.

The sintered structure is shown in Figs. 7 and 8.

The hardness of the cemented carbide component may be about 1390 to about 1400 HV30 (IS03878), the toughness (Klc) being about 8.6 to about 9.3 MPa ●√m using Palmqvist toughness technique according to ISO28079 and a density of about 10.02 to about 10.17 g/cm³.

The grades disclosed herein demonstrate improved corrosion resistance in comparison to a standard seal ring grade. Corrosion resistance was determined using a modified test to ASTM G61. ASTM G61 covers a procedure for conducting potentiodynamic polarization measurements. The modification of this standard has been in the media used. Instead of using 3.5% NaCl solution in the tests, artificial seawater according to ASTM DI141 was used as the media. Furthermore, the flushed port cell used in ASTM G61 was replaced by sealing the specimen with epoxy to avoid crevice corrosion on the edge of the sample.

The pitting potential was used as a measure for comparison. The higher the value the better the corrosion resistance of the material. The value measured for a standard seal ring grade was Epit=263mV SCE. However, for the LW grade Epit=318mV SCE showing improved corrosion resistance.

**Table 2**

| Ref | A (illustrative only) | B (illustrative only) | C (encompassed by the present invention) | D (encompassed by the present invention) |
|---|---|---|---|---|
| Sample | LW flow control | LW seal ring | LW + CR seal | LW + CR seal ring |
| WC (wt%) | balance | 63.2 | 66.04 | 62.79 |
| WC grain size (µm) | 0.8 | 4.0 - 8.0 | 1.05 - 1.15 | 1.05 - 1.15 |
| TiC (wt%) | 21 | 20.8 | 21.95 | 20.86 |
| Co (wt%) | 8.3 | 8.2 | 0 | 0 |
| Ni (wt%) | 5.7 | 5.6 | 10.11 | 13.78 |
| Mo (wt%) | 0.2 | 0.2 | 0.95 | 1.29 |
| Cr₃C₂ (wt%) | 2 | 2 | 0.95 | 1.29 |

**Table 3**

| Ref | A | C | D |
|---|---|---|---|
| Sample | LW flow control | LW + CR seal ring | LW + CR seal ring |
| Density (gm/cm³) | 9.8 - 10 | 10.2 | 10.02 - 10.17 |
| Hardness (Hv30) | 1350 - 1500 | 1550 | 1390 - 1400 |
| Toughness (Klc) | 9.5 | 8.5 - 9.5 | 8.6 - 9.3 |

## Claims

1. A cemented carbide for fluid handling components and seal rings, the cemented carbide having a composition comprising:
15 to 30wt% TiC;
5 to 20wt% Ni;
0.5 to 2.5wt% Cr₃C₂;
0.7 to 1.6wt% Mo; and
the remainder WC.

2. The cemented carbide for fluid handling components and seal rings of claim 1, wherein the composition comprises from 20 to 23 wt % TiC.

3. The cemented carbide for fluid handling components and seal rings of claim 1 or claim 2, wherein the composition comprises from 0.8 to 1.5 wt % Cr₃C₂.

4. The cemented carbide for fluid handling components and seal rings according to any of claims 1-3, wherein the composition comprises from 9.5 to 14.5 wt% Ni.

5. The cemented carbide for fluid handling components and seal rings according to any of claims 1-4, wherein cemented carbide composition has an average WC grain size of from 0.9 µm to 1.3 µm as measured by FSSS.

## Patentansprüche

1. Zementiertes Carbid für Flüssigkeitshandhabungskomponenten und Dichtungsringe, wobei das zementierte Carbid eine Zusammensetzung aufweist, die umfasst:
15 bis 30 Gew. -% TiC;
5 bis 20 Gew. -% Ni;
0,5 bis 2,5 Gew. -% Cr₃C₂;
0,7 bis 1,6 Gew.-% Mo; und
zum Rest WC.

2. Zementiertes Carbid für Flüssigkeitshandhabungskomponenten und Dichtungsringe nach Anspruch 1, wobei die Zusammensetzung von 20 bis 23 Gew.-% TiC umfasst.

3. Zementiertes Carbid für Flüssigkeitshandhabungskomponenten und Dichtungsringe nach Anspruch 1 oder Anspruch 2, wobei die Zusammensetzung von 0,8 bis 1,5 Gew.-% Cr₃C₂ umfasst.

4. Zementiertes Carbid für Flüssigkeitshandhabungskomponenten und Dichtungsringe nach einem der Ansprüche 1 bis 3, wobei die Zusammensetzung von 9,5 bis 14,5 Gew.-% Ni umfasst.

5. Zementiertes Carbid für Flüssigkeitshandhabungskomponenten und Dichtungsringe nach einem der Ansprüche 1 bis 4, wobei die zementierte Carbidzusammensetzung eine durchschnittliche WC-Korngröße von 0,9 µm bis 1,3 µm aufweist, gemessen per FSSS.

## Revendications

1. Carbure cémenté pour composants de manipulation de fluide et bagues d'étanchéité, le carbure cémenté ayant une composition comprenant :
15 à 30 % en poids de TiC ;
5 à 20 % en poids de Ni ;
0,5 à 2,5 % en poids de Cr₃C₂ ;
0,7 à 1,6 % en poids de Mo ; et
du WC pour le reste.

2. Carbure cémenté pour composants de manipulation de fluide et bagues d'étanchéité selon la revendication 1, dans lequel la composition comprend 20 à 23 % en poids de TiC.

3. Carbure cémenté pour composants de manipulation de fluide et bagues d'étanchéité selon la revendication 1 ou la revendication 2, dans lequel la composition comprend 0,8 à 1,5 % en poids de Cr₃C₂.

4. Carbure cémenté pour composants de manipulation de fluide et bagues d'étanchéité selon l'une quelconque des revendications 1 à 3, dans lequel la composition comprend 9,5 à 14,5 % en poids de Ni.

5. Carbure cémenté pour composants de manipulation de fluide et bagues d'étanchéité selon l'une quelconque des revendications 1 à 4, dans lequel la composition du carbure cémenté a une granulométrie moyenne du WC, telle que mesurée par FSSS, de 0,9 µm à 1,3 µm.
